

No. 683,851.

Patented Oct. 1, 1901.

C. CRONENBERG.  
COMPOUND FOR THERMAPHORES.

(Application filed Feb. 4, 1899.)

(No Model.)



Witnesses

Daniel B. Sniger  
J. W. Grover

Inventor

Carl Cronenbergs.  
By  
B. Sniger.  
Attorney

# UNITED STATES PATENT OFFICE.

CARL CRONENBERG, OF BERLIN, GERMANY.

## COMPOUND FOR THERMAPHORES.

SPECIFICATION forming part of Letters Patent No. 683,851, dated October 1, 1901.

Application filed February 4, 1899. Serial No. 704,521. (No specimens.)

*To all whom it may concern:*

Be it known that I, CARL CRONENBERG, merchant, a subject of the Emperor of Germany, residing at 187 Friedrichstrasse, Berlin, in the Kingdom of Prussia and Empire of Germany, have invented certain new and useful Improvements in Compounds for Thermaphores, of which the following is a full, clear, and exact description.

10 This invention relates to improvements in compounds for thermaphores or that class of apparatus in which heat is generated by melting sodium acetate.

In the accompanying drawing I have shown 15 in vertical section a form of apparatus or thermaphore in which my compound is adapted for use.

In the employment of such apparatus when a certain quantity of heat has to be maintained for a long time by the salts which have been previously melted and are to be again crystallized several points have to be observed in order to insure satisfactory results. For instance, it is necessary after the melting 25 of the crystalline substance that the recrystallization—that is to say, the giving of the heat—can be set in progress at the time when required for use, and that, further, for the protection of the sides of the vessel and 30 for other practical reasons the crystallized material should not settle down into a solid body, but rather assume the form of a pulp or semiliquid. The first of these objects is attained as follows: The more or less concentrated 35 solution of salts, chiefly consisting, as is known, of acetate of sodium, is inclosed in a hollow receptacle the opening of which is closed by means of an air-tight screw-cover Z, having in its under side a pointed rod 40 which projects into the crystalline substance. As the vessel is not entirely filled, there is a free space of about ten millimeters in height above the body of the salts. The advantage of this arrangement is that in the recrystallization 45 of the salts the crystalline material takes on a form resembling sand in consistency and has space for expansion, whereby injury to the vessel is avoided. If the heating

vessel B, which may be of any desired construction, be heated for the purpose of melting the salts, the very slow and first recrystallization which takes place after the removal from the source of heat may be employed for heating any desired substance contained in a vessel inclosed in said hollow receptacle. After the cooling, which proceeds very slowly, a complete recrystallization of the salts does not set in without special action from without. Even an ordinary shock or vibration is without effect on the salt solution contained in the particular vessel. The recrystallization or giving off of the heat begins, however, if the hitherto closed screw-cover be opened and thereby the point of the rod which is in the liquid be partially withdrawn therefrom. The complete crystallizing of the salts employed occurs immediately, and the heat thereby set free can be applied for various purposes.

For the employment of this kind of heat-preserving apparatus with metal or sheet-metal vessels it is of importance for the protection of the sides and of still greater importance in the employment of this heat-preserving apparatus with flexible sides that the body of salts be not reduced to a compact form in crystallizing, but that it should have a soft pliable texture. For attaining this object a certain quantity of glycerin is added to the solution of salts, through the addition of which the body of salts in crystallizing is prevented from settling down in compact form, but assumes the consistency of moist sand, which is yielding and will conform to the shape of the container or vessel.

What I claim, and desire to secure by Letters Patent, is—

A compound for thermaphores, composed of acetate of soda and glycerin.

In witness whereof I subscribe my signature in presence of two witnesses.

CARL CRONENBERG.

Witnesses:

ERWIN L. GOLDSCHMIDT,  
HENRY HASPER.